

# United States Patent [19]

Doin et al.

[11] 3,912,561

[45] Oct. 14, 1975

[54] PYROTECHNIC COMPOSITIONS FOR GAS GENERATION

[75] Inventors: **Bernard J. Doin**, Saint Medard en Jalles; **Jean P. Thomas**, Paris, both of France

[73] Assignee: **Societe Nationale des Poudres et Explosifs**, Paris, France

[22] Filed: **Oct. 9, 1973**

[21] Appl. No.: **404,762**

[30] Foreign Application Priority Data

Oct. 17, 1972 France ..... 72.36738

[52] U.S. Cl. ..... 149/35; 149/85; 149/2

[51] Int. Cl. <sup>2</sup> ..... C22C 37/00

[58] Field of Search ..... 149/35, 85, 2

[56] References Cited

UNITED STATES PATENTS

3,785,674 1/1974 Poole et al. .... 149/35 X

3,797,854 3/1974 Poole et al. .... 149/35 X

Primary Examiner—Stephen J. Lechert, Jr.  
Attorney, Agent, or Firm—Bucknam and Archer

[57]

## ABSTRACT

A gas-generating pyrotechnic composition comprises:  
a. a fuel selected from the group consisting of alkali metal azides and alkaline earth metal azides,  
b. an alkali metal oxidant selected from the group consisting of alkali metal perchlorates and bichromates,  
c. a nitrogenous compound selected from the group consisting of aminotetrazole, aminotetrazole hydrate, azodicarbonamide and azotetrazole, and  
d. optionally, silica as an additive for reacting with the solid combustion residues of the composition.

Such compositions are particularly intended for the deployment of inflatable safety devices for driver and passenger protection in automobiles and other fast vehicles.

12 Claims, No Drawings

## PYROTECHNIC COMPOSITIONS FOR GAS GENERATION

The present invention is concerned with pyrotechnic compositions which generate combustion gases which are substantially non-toxic and which can be used, in particular, for the deployment of inflatable safety devices designed to protect the drivers and passengers of motor vehicles and other fast vehicles.

Propellant compositions are known containing, as an additive, a small percentage of an azide, such as sodium azide, or of a tetrazole derivative, such as aminotetrazole, but on combustion, these compositions, which are primarily intended for the propulsion of rockets, generate a substantial volume of toxic gases.

Propellant compositions based on a mixture of an azide, such as sodium azide, and an inorganic oxidant, such as potassium perchlorate, and, optionally, a small percentage of an inorganic oxide, such as silica, as combustion catalyst, are also known. However, these compositions have only a limited yield of gas unless the mixture is so formulated as to provide a substantially stoichiometric quantity of oxygen which, in turn, leads to the production of toxic nitrogen oxides in the combustion gases. These propellant compositions are, however, primarily intended for the propulsion of rockets, for which purpose the production of such nitrogen oxides is not disadvantageous.

Gas-generating compositions have also been proposed which enable a large volume of non-toxic gas to be obtained in a very short period. These compositions comprise an inorganic oxidant and a plastics binder and produce combustion gases containing a relatively high proportion of oxygen. The latter characteristic could be a disadvantage when such compositions are used for the deployment of inflatable safety devices in case of accidents in view of the risk of fire.

We have now developed a gas-generating pyrotechnic composition which gives, on combustion, a high yield of substantially non-toxic gas at a moderate temperature and within a very short period. The combustion gases obtained, predominantly consist of nitrogen, a non-reactive gas, and have a low oxygen content and, in addition, the solid combustion residues are physiologically harmless.

According to the present invention, we provide a gas-generating pyrotechnic composition, which comprises:

- a. a fuel consisting of an alkali metal azide or alkaline earth metal azide,
- b. an alkali metal oxidant selected from alkali metal perchlorates and bichromates,
- c. a nitrogenous compound selected from aminotetrazole, aminotetrazole hydrate, azocarbonamide and azotetrazole, and
- d. optionally, silica as an additive for reacting with the solid combustion residues of the composition.

In preferred compositions according to the invention, the weight ratio of azide: alkali metal oxidant is greater than 1 and the weight ratio nitrogenous compound: azide is less than 48%.

The composition preferably comprises, by weight:

- a. 50 to 80 parts of sodium azide,
- b. 50 to 20 parts of potassium perchlorate, for a total of 100 parts of azide and perchlorate,
- c. up to 48%, with respect to the azide, of aminotetrazole or aminotetrazole hydrate, and
- d. at least 6%, with respect to the azide, of silica.

The solid combustion residues of the composition according to the invention comprise alkali metal or alka-

line earth metal oxides, most of which have an irritating physiological action and can cause burns, particularly when the constituents (a) and (b) are sodium azide and potassium perchlorate, respectively. The incorporation of silica in the composition enables these oxides to be suppressed by converting them into silicates which have no physiological action on the organism. For example, the total suppression of sodium oxide in the combustion residues is obtained by using 9.3% of silica with respect to the quantity of sodium azide; in practice, an amount of silica greater than 6% enables a partial, but satisfactory, suppression of sodium oxide to be obtained.

The presence of one or more of the specified nitrogenous compounds in the compositions according to the invention gives rise to the following advantages as compared with known gas-generating pyrotechnic compositions:

- i. the compositions according to the invention have a shorter ignition time, of the order of several milliseconds, while retaining a sufficiently high selfignition temperature for the composition to be completely safe in use;
- ii. the yield of gas from the compositions according to the invention (expressed in litres per gram) is considerably greater and the combustion gases consist predominantly of nitrogen; and
- iii. the potential expressed in cal/g, and the combustion temperature, are lower.

In addition, while the combustion gases obtained from the compositions according to the invention contain some carbon monoxide, the proportion of the latter can be kept below the critical toxic value and the combustion gases contain substantially less toxic nitrogen oxides than the gases obtained from known gas-generating pyrotechnic compositions. Since the combustion gases obtained from the composition according to the invention are particularly intended for the deployment of inflatable safety devices, for which purpose the gases should be at only a moderate temperature, it is of particular importance to obtain:

- i. the lowest possible combustion temperature, since the combustion gases have to be cooled before their introduction into the inflatable device,
- ii. a maximum yield of gas and a very short ignition period, since for safety devices the time of inflation is usually required to be no longer than about 20 milliseconds, and
- iii. a minimum toxicity, which requires a reduction in the amount of nitrogen oxides, the latter being much more dangerous than carbon monoxide.

In the case of compositions comprising sodium azide, potassium perchlorate, and aminotetrazole hydrate, which has a potential of about 200 cal/g and which yields, on combustion, 0.5 litre of nitrogen per gram, together with water vapour and a small quantity of hydrogen, if it is desired to obtain combustion gases in which the carbon monoxide content does not exceed about 100 parts per million, the maximum content of aminotetrazole hydrate in the composition is defined by the following conditions, all parts and proportions being by weight:

$$\text{for } \frac{\text{Na}_3}{\text{KClO}_4} = \frac{70}{30}, \text{ the ratio } \frac{\text{aminotetrazole}}{\text{Na}_3} \text{ should be}$$

less than  $\frac{6}{70}$ , i.e. less than 8.5%

## -Continued

for  $\frac{\text{NaN}_3}{\text{KClO}_4} = \frac{60}{40}$ , the ratio  $\frac{\text{aminotetrazole}}{\text{NaN}_3}$  should be less than  $\frac{16}{60}$ , i.e. less than 27%

for  $\frac{\text{NaN}_3}{\text{KClO}_4} = \frac{50}{50}$ , the ratio  $\frac{\text{aminotetrazole}}{\text{NaN}_3}$  should be less than  $\frac{24}{50}$ , i.e. less than 48%

When a composition diagram is constructed in which the ordinates represent the weight ratio  $\text{NaN}_3/\text{KClO}_4$  and the abscissae the weight ratio aminotetrazole/ $\text{NaN}_3$ , the curve passing through the three points, a, b and c, defined as follows:

|           |                                              |                       |                       |                       |
|-----------|----------------------------------------------|-----------------------|-----------------------|-----------------------|
| ordinates | $\text{NaN}_3/\text{KClO}_4$                 | <sup>a</sup><br>70/30 | <sup>b</sup><br>60/40 | <sup>c</sup><br>50/50 |
| abscissae | $\frac{\text{Aminotetrazole}}{\text{NaN}_3}$ | 85%                   | 27%                   | 48%                   |

delimits a region situated below the curve, in which the amount of carbon monoxide in the combustion gases does not exceed about 100 ppm.

In addition, given that ignition difficulties are encountered when the ratio  $\text{NaN}_3/\text{KClO}_4$  is less than 1, the region representing the most preferred compositions is that lying between the curve defined by the three points a, b and c, the ordinate axis, and the straight line parallel to the abscissae axis for which the ordinate value = 1, corresponding to equal amounts of potassium perchlorate and sodium azide.

In the following examples reference will be made, for the purpose of comparison, to three gas-generating pyrotechnic compositions illustrative of the prior art and containing only sodium azide, potassium perchlorate and silica. The formulation of these compositions, in parts by weight, was as follows:

| Composition     | A   | B   | C   |
|-----------------|-----|-----|-----|
| $\text{NaN}_3$  | 50  | 60  | 70  |
| $\text{KClO}_4$ | 50  | 40  | 30  |
| $\text{SiO}_2$  | 4.6 | 5.6 | 6.5 |

(average particle size  $30\mu$ ).

The potentials obtained experimentally with these compositions decreased as the amount of perchlorate decreases, and were equal to: 1330 cal/g, 1270 cal/g and 1220 cal/g for compositions A, B and C respectively.

The self-ignition temperature of the three compositions was  $415^\circ\text{C}$ .

The gas yield was from 0.248 l/g and 0.356 l/g (the gases being at normal pressure and temperature) and the combustion gases contained from 96% to 99.5% of nitrogen mass of the combustion gases. The elimination of sodium oxide in the solid combustion residues was satisfactory due to the presence of powdered silica in the indicated quantities.

The use of other alkali metal azides or other alkaline earth metal azides and of other alkali metal perchlorates or bichromates gives different, but comparable, values and results. Compositions A, B, C show the importance of using large amounts of azide, since, on the one hand, the combustion temperature, which is related to the potential of the composition, decreases and, on the other hand, the yield of gases increases, but concomitantly the formation of nitrogen oxides also increases and, for example, in the range of proportions comprised between

$$\frac{70}{30} < \frac{\text{NaN}_3}{\text{KClO}_4} < \frac{80}{20}$$

15

the compositions of the prior art type have a higher toxicity due to the excessive formation of nitrogen oxides.

The present invention is illustrated by the following examples in which all parts and percentages are by weight.

## EXAMPLES

Pyrotechnic compositions having the following formulations were prepared and formed into pellets:

| Composition                                                     | D  | E    | F   | G    |
|-----------------------------------------------------------------|----|------|-----|------|
| $\text{NaN}_3$                                                  | 60 | 60   | 50  | 50   |
| $\text{KClO}_4$                                                 | 40 | 40   | 50  | 50   |
| aminotetrazole                                                  | 16 | 18   | 24  | 28   |
| Characteristics                                                 |    |      |     |      |
| Toxicity of the combustion gases expressed in parts per million |    |      |     |      |
| Carbon monoxide                                                 | 50 | 1100 | 90  | 2100 |
| Nitrogen oxides                                                 | 80 | 30   | 110 | 45   |

The potentials and combustion rates of these compositions were lower than those of compositions A, B and C having the same  $\text{NaN}_3/\text{KClO}_4$  ratio. The potentials obtained were about the order of 1000 cal/g and the gaseous yields were about 0.45 l/g (at normal pressure and temperature).

The use of other specified nitrogenous compounds, that is aminotetrazole hydrate, azodicarbonamide and azotetrazole, gives different, but comparable, values and the effects observed are similar.

By way of comparison, there are given below the combustion characteristics of two compositions comprising only sodium azide and potassium perchlorate.

|                   |                 |                                              |
|-------------------|-----------------|----------------------------------------------|
| Composition II    | $\text{NaN}_3$  | 50 parts                                     |
|                   | $\text{KClO}_4$ | 50 parts                                     |
| Aluminum stearate |                 | 3 parts (necessary for formation of pellets) |
| Characteristics   |                 |                                              |
| Gas yield         |                 | 0.288 l/g                                    |
| Combustion rate   |                 | 80 mm/s at 34 bars                           |
| Composition I     |                 |                                              |
| $\text{NaN}_3$    |                 | 70 parts                                     |
| $\text{KClO}_4$   |                 | 30 parts                                     |
| Aluminum stearate |                 | 3 parts                                      |
| Characteristics   |                 |                                              |
| Gas yield         |                 | 0.356 l/g                                    |
| Gases produced    |                 | $\text{O}_2$ 0.8%<br>$\text{N}_2$ 99.2%      |
| Combustion rate   |                 | 350 mm/s at 80 bars.                         |

The following example illustrates the employment of aminotetrazole and silica in a gas-generating pyrotechnic composition according to the invention.

| Composition K                                   | (in the form of pellets) |
|-------------------------------------------------|--------------------------|
| $\text{NaN}_3$                                  | 70 parts                 |
| $\text{KClO}_4$                                 | 30 parts                 |
| aminotetrazole                                  | 6.5 parts                |
| $\text{SiO}_2$ (average particle size $30\mu$ ) | 6.5 parts                |

The combustion characteristics obtained with this composition were as follows:

|                                                           |                                                                                        |
|-----------------------------------------------------------|----------------------------------------------------------------------------------------|
| Gas yield                                                 | 0.45 l/g                                                                               |
| Gases produced                                            | $\text{N}_2 = 83\%$<br>$\text{H}_2 = 16\%$                                             |
|                                                           | Various non-toxic gases: 1%                                                            |
| Solid residues                                            | $\text{KCl}$<br>$\text{Na}_2\text{O}_2$<br>$\text{Na}_2\text{SiO}_3$<br>$\text{SiO}_2$ |
| Temperature of the gases on release read by thermocouple: | 500°C                                                                                  |
| Potential:                                                | about 1000 cal/g                                                                       |
| Combustion rate:                                          | 280 mm/s at 40 bars.                                                                   |

In the foregoing examples, the preparation of the pyrotechnic compositions according to the invention is effected in a conventional manner by mixing of the constituents. Shaped charges can be formed by incorporating a suitable binder and subjecting the composition to a conventional pelleting or extrusion operation. Various shapes can be used according to the firing characteristics required. By way of example, compositions containing from 1 to 2 parts by weight of a metal stearate and in the form of pellets of 9.5 mm diameter and 3 mm thickness, are suitable.

The constituents are preferably physically treated to select a particular particle size fraction and/or to eliminate moisture. For example, potassium perchlorate is preferably dried at 80°C for 12 hours and sodium azide is preferably crushed by rollers to pass through a  $295\mu$  screen. The mixing should be carried out to obtain a mixture which is powdery and apparently homogeneous. Simultaneous introduction of the constituents into a mixer, such as a V mixer (Moritz), and mixing for 1 hour is suitable in most cases.

When pellets are required, pelletising of the powder mixture is preferably effected under the following working conditions in, for example a pelletiser of the Stokes type:

|                     |                                                                   |
|---------------------|-------------------------------------------------------------------|
| Pelleting pressure: | 2 to 10 tonnes/cm <sup>2</sup>                                    |
| Moisture content:   | 30% to 40%                                                        |
| Temperature:        | 21 to 29°C                                                        |
| Binder:             | aluminum stearate, polytetrafluoroethylene, or potassium bromide. |

We claim:

1. A gas-generating pyrotechnic composition, which comprises:

- a fuel selected from the group consisting of alkali metal azides and alkaline earth metal azides,
- an alkali metal oxidant selected from the group consisting of alkali metal perchlorates and bichromates,
- a nitrogenous compound selected from the group consisting of aminotetrazole, aminotetrazole hydrate, azodicarbonamide and azotetrazole.

2. The composition according to claim 1 additionally comprising silica.

3. A composition as set forth in claim 1, wherein the weight ratio of azide: alkali metal oxidant is greater than 1.

4. A composition as set forth in claim 1, wherein the weight ratio of nitrogenous compound: azide is less than 48%.

5. A composition as set forth in claim 2, which comprises:

- sodium azide,
- potassium perchlorate,
- a nitrogenous compound selected from the group consisting of aminotetrazole and aminotetrazole hydrate, and
- silica.

15 6. A composition as set forth in claim 2, which comprises, by weight:

- 50 to 80 parts of sodium azide,
- 50 to 20 parts of potassium perchlorate, for a total of 100 parts of azide and perchlorate,
- up to 48%, with respect to the azide, of a nitrogenous compound selected from the group consisting of aminotetrazole and aminotetrazole hydrate, and
- at least 6%, with respect to the azide, of silica.

20 7. A composition as set forth in claim 6, which comprises, by weight, about 9.3% of silica with respect to the azide.

8. A composition as set forth in claim 6, which comprises, by weight:

- 50 to 60 parts of sodium azide,
- 50 to 40 parts of potassium perchlorate, for a total of 100 parts of azide and perchlorate, and
- 28 to 48%, with respect to the azide, of a nitrogenous compound selected from the group consisting of aminotetrazole and aminotetrazole hydrate.

25 9. A composition as set forth in claim 6, which comprises, by weight:

- about 70 parts of sodium azide,
- about 30 parts of potassium perchlorate,
- about 6.5 parts of a nitrogenous compound selected from the group consisting of aminotetrazole and aminotetrazole hydrate, and
- about 6.5 parts of silica.

30 10. A composition as set forth in claim 5, in which the weight ratios  $\text{NaN}_3/\text{KClO}_4$  and aminotetrazole/ $\text{NaN}_3$  fall within the region on a composition diagram in which the ratio  $\text{NaN}_3/\text{KClO}_4$  is plotted as the ordinates and the ratio aminotetrazole/ $\text{NaN}_3$  as the abscissae, defined by

i. the curve passing through three points, a, b and c, which are respectively defined as follows:

$$a, \frac{\text{NaN}_3}{\text{KClO}_4} = \frac{70}{30}, \frac{\text{aminotetrazole}}{\text{NaN}_3} = \frac{6}{70}$$

$$b, \frac{\text{NaN}_3}{\text{KClO}_4} = \frac{60}{40}, \frac{\text{aminotetrazole}}{\text{NaN}_3} = \frac{16}{60}$$

$$c, \frac{\text{NaN}_3}{\text{KClO}_4} = \frac{50}{50}, \frac{\text{aminotetrazole}}{\text{NaN}_3} = \frac{24}{50}$$

ii. the straight line parallel to the abscissae axis for which the ordinate value = 1, and

iii. the axis of the ordinates.

35 11. A composition as set forth in claim 2, in the form of pellets.

12. A composition as set forth in claim 11, wherein said pellets comprise a binder selected from the group consisting of aluminium stearate, polytetrafluoroethylene and potassium bromide.

\* \* \* \* \*